

Patented Mar. 6, 1928.

1,661,606

# UNITED STATES PATENT OFFICE.

AUGUSTE ESCAICH AND JEAN PAUL WORMS, OF PARIS, FRANCE.

## DYEING PROCESS.

No Drawing. Application filed November 20, 1923, Serial No. 675,956, and in Germany November 25, 1922.

This invention relates to a dyeing process applicable to all fibres, leathers, hairs and the like which consists in causing reducing agents to act in either the hot or cold state in an acid medium on ferri and ferrocyanides and in the presence of traces of catalyzing salts or of metallic oxides. By ferro and ferricyanides, we mean in this specification, the double cyanides of iron and of an alkali metal, sodium or potassium.

These substances can furnish various colors. They have, moreover, been used for a long time, for giving blue (Raymond, Prussian, French blue etc.).

It is well known that for obtaining these blues one generally uses somewhat considerable amounts of minerals acids, in a first operation, and tin salts which are relatively of a high price, in a subsequent operation.

In the present process use is made of the fact that potassium ferricyanide, in the presence of various reducing agents will dye any fibres very easily if the medium is slightly acid and contains traces of catalyzing mercury compounds.

The best results are obtained by acid mercury sulphate, known as Denigès reagent consisting of yellow mercury oxide 50 gr., sulphuric acid 200 c. c., distilled water 1000 30 c. c. the amount of mercury oxide may however be increased.

The reducers suitable for use are numerous and will be enumerated hereinafter, for instance, ordinary sugar may be employed as follows:-

20 litres of water +50 c. c. of a solution of sugar, at 10% +40 c. c. of a solution of acid mercury sulphate; is brought to the boil in order to invert the sugar, and then 40 c. c. of a solution of 10 potassium ferri-

cyanide for 100 water is added; fabrics of any kind immersed at the beginning or at the end in the bath, will be colored blue. With the above proportions, the color is

very marked on wool, less intense on silk and cotton, but is sufficient for light shades.

It is thus possible to develop very interesting colors with very reduced quantities of alkali metal ferro or ferricyanides and of mineral acid.

The composition of the bath remaining otherwise the same, by doubling the ferri-cyanide, that is to say, 80 c. cm. at 10% for 20 litres of water; a blue which is deep 55 on wool and very decided on silk is obtained.

The same results are obtained with cold treatment in about 24 hours.

With hot treatment, the first stage of coloring of the fabrics results below boiling-point temperature in greens. If desired, with a view to shading, the operation can be stopped at this point before proceeding to the blue stage.

In the absence of sugar, the mercury sulphate and the ferricyanide give a blue of less depth.

The sugar can be replaced by equivalent quantities of glucose.

If, theoretically, in an alkaline medium, the reduction of two molecules of ferricyanide is obtained with a molecule of glucose, in practice practically equal quantities of these two substances can be used. In acid medium the proportions hereinbefore indicated give excellent results.

Ferrocyanide substituted for ferricyanide gives lighter colors. With a view to producing a shade or tint, these two substances can be mixed at the rate of 1 part of ferricyanide and of 1 to 10 parts of ferrocyanide. With these proportions the addition of ferric chloride or sulphate gives very fine blues.

Instead of sugar, various reducers can be employed and used in an amount equal to that of the ferricyanide or to a smaller amount if the conditions of solubility or of economy are in favour of a decrease.

In a quantity equal to that of the ferrocyanide use can be made of commercial formic acid, hydroquinone, resorcin, formaldehyde, dextrine, soluble starch, aniline salts, and tannins; in a smaller quantity one will use the naphthols (0.50 gr. per liter of bath), the pyrocatechin of saponin (0.50 gr. for 1 liter).

The colors are especially good when formic acid, naphthols, hydroquinone or resorcin are used.

The tannins are employed, either dissolved in very small quantities in the bath, or previously fixed as mordants on the fibre in the ordinary manner. They adapt themselves to all the operations of dulling, bluing, passing into black charging, etc., practiced in the known processes with prussiates.

Saponin is very suitable as many Algerian or Moorish wools are bleached by means of local soap-worts of which the *Saponaria vaccaria* (Morocco Tirestre) contains from 8 to 15% of saponin. European soap-worts, Panama wood may be substituted for the

sugar and has the advantage of "drawing" very uniformly. Further it must be borne in mind that the saponin seems to adhere to the fibre like a tannic mordant and under 5 the same conditions, which allows of dyeing blue after washing the fabric by immersion in the bath. Hence only two reagents will be required in the bath, the acid mercury sulphate and the ferricyanide, the reducer 10 being carried by the saponified fibre.

If the reducer employed is itself a chromogen (tannin, naphthols) and is fixed as a mordant on the fibre, it will be possible to alter the blue tint obtained by passing a 15 previously tanned blue fibre into a bath of molybdate or a blue fibre previously naphtholated into a bath of nitrous acid.

We claim—

1. Method of dyeing any fibres with the

aid of a double cyanide of iron and of an alkali metal, consisting in causing to act on the fibres a slightly acid bath containing a double cyanide of iron and of an alkali metal, an organic reducing agent and traces of a mercury compound.

2. Method of dyeing any fibres with the aid of a double cyanide of iron and of an alkali metal, consisting in causing to act on the fibres a slightly acid bath containing a ferricyanide of an alkali metal, a ferrocyanide of an alkali metal, an organic reducing agent and traces of a mercury compound.

In testimony, that we claim the foregoing as our invention, we have signed our names.

AUGUSTE ESCAICH.  
JEAN PAUL WORMS.